

# United States Patent Office

3,361,652

Patented Jan. 2, 1968

## 1

3,361,652

**ELECTRODEPOSITION OF BRIGHT TIN**  
 Joachim Korpüün, Friedrich Sedlacek, and Joachim Steeg,  
 Geislingen an der Steige, Germany, assignors to Dr. Ing.  
 Max Schlotter, Geislingen an der Steige, Germany, a  
 firm  
 No Drawing. Filed Aug. 24, 1964, Ser. No. 391,790  
 Claims priority, application Germany, Aug. 28, 1963,  
 Sch 33,772; Aug. 5, 1964, Sch 35,588  
 16 Claims. (Cl. 204—54)

## ABSTRACT OF THE DISCLOSURE

Semi-bright or bright tin electrodeposits are formed in otherwise conventional acid tin baths in the presence of a dissolved primary brightener of the formula



in which X is phenyl, furfuryl, or pyridyl and Y may be hydrogen, formyl, carboxyl, alkyl, hydroxylalkyl, formylalkyl, or the acyl radical of a carboxylic acid. Formaldehyde and certain imidazoline derivatives act as secondary brighteners, particularly when employed with nonionic wetting agents.

This invention relates to a method of electrodepositing bright tin, and to an acid solution suitable as an aqueous electrolyte for performing the method.

Commercially used bright acid tin plating solutions contain as brighteners tar and tar fractions obtained in the destructive distillation of wood. Such electrolytes are difficult to control, and it is not readily possible to produce bright tin plates of consistent quality from them over extended periods of time.

We have found a group of primary brighteners for acid tin plating electrolytes which perform reliably over extended periods of operation, and yield semi-bright or fully bright deposits in a reproducible manner. The primary brighteners of the invention cooperate with secondary brighteners which improve brightness and/or widen the cathode current density range in which the deposits have the desired brightness.

Wetting agents are employed in the acid tin plating solutions of the invention. Non-ionic wetting agents are preferred, and the water soluble ether of polyglycols which are readily available are both effective and stable under the normal operating conditions of the electrolyte. They may have from ten to thirty ethyleneoxy radicals per molecule, the molecular weight being mainly limited by considerations of solubility.

The primary brighteners of the invention are soluble ethylene derivatives of the formula  $X-\text{CH}=\text{CH}-Y$  wherein X is phenyl, furfuryl or pyridyl, and Y may be hydrogen, formyl, carboxyl, alkyl, hydroxylalkyl, formylalkyl, or the acyl radical of a carboxylic acid, the nature of the substituents being limited mainly by the requirement that the brightener be soluble in the electrolyte in effective amounts.

The following examples are representative of compounds which are adequately soluble in the acid electrolytes of the invention:

Styrene— $\text{C}_6\text{H}_5-\text{CH}=\text{CH}_2$

Cinnamyl alcohol— $\text{C}_6\text{H}_5-\text{CH}=\text{CH}-\text{CH}_2\text{OH}$

Cinnamic acid— $\text{C}_6\text{H}_5-\text{CH}=\text{CH}-\text{COOH}$

Cinnamaldehyde— $\text{C}_6\text{H}_5-\text{CH}=\text{CH}-\text{CHO}$

o-Methoxycinnamic acid—

$\text{CH}_3\text{O}-\text{C}_6\text{H}_4-\text{CH}=\text{CH}-\text{COOH}$

## 2

3-furylacrylic acid— $\text{C}_4\text{H}_3\text{O}-\text{CH}=\text{CH}-\text{COOH}$   
 Benzylideneacetone— $\text{C}_6\text{H}_5-\text{CH}=\text{CH}-\text{CO}-\text{CH}_3$   
 Curcumin—

5  $[\text{C}_6\text{H}_3(\text{OH})(\text{OCH}_3)-\text{CH}=\text{CH}-\text{CO}]_2:\text{CH}_2$

4-(2-furyl)-3-butene-2-one—

$\text{C}_4\text{H}_3\text{O}-\text{CH}=\text{CH}-\text{CO}-\text{CH}_3$

4-p-sulfophenyl-3-butene-2-one—

10  $\text{C}_6\text{H}_4(\text{SO}_3\text{H})-\text{CH}=\text{CH}-\text{CO}-\text{CH}_3$

1,5-di-p-sulfophenyl-1,4-pentadiene-3-one—

$[\text{C}_6\text{H}_4(\text{SO}_3\text{H})-\text{CH}=\text{CH}]_2:\text{CO}$

2-pentyl-3-phenyl-propenal—

$\text{C}_6\text{H}_5-\text{CH}=\text{CH}-(\text{CH}_2)_5-\text{CHO}$

4-hydroxy-3-methoxy-benzylideneacetone—

$\text{C}_6\text{H}_3(\text{OH})(\text{OCH}_3)-\text{CH}=\text{CH}-\text{CO}-\text{CH}_3$

20 4-(pyridyl-2)-3-butene-2-one—

$\text{C}_5\text{H}_4\text{N}-\text{CH}=\text{CH}-\text{CO}-\text{CH}_3$

As is evident from the examples listed above, the length of carbon chains attached to the ethylene core of the brightening agent does not interfere with the brightening effect as long as adequate solubility is maintained, nor are substituents in the radicals X and Y of importance as long as they do not affect the stability of the brightener in a harmful manner.

25 30 The primary brighteners are listed in part in the Merck Index, 7th ed., with their methods of preparation. The compounds not listed in the Index may be prepared according to the following publications:

o-Methoxycinnamic acid: J. Chem. Soc. (London) 31, 35 414 (Perkin);

4-(2-furyl)-3-butene-2-one; Ber. 14, 1459 (Schmidt);  
 4-phenyl-3-butene-2-one-1-sulfonic acid and 1,5-di-  
 phenyl-1,4-pentadiene-4-one-2,4-disulfonic acid: Zentral-  
 blatt 1954, p. 1927;

40 2-pentyl-3-phenyl-propenal: Comptes Rendus 237 (1953) 1012 (Durr);

4-hydroxy-3-methoxy-benzylideneacetone: J. Chem. Soc. (London) 1938, p. 1568 (Nisbet); and

4-(pyridyl-2)-3-butene-2-one: Zentralblatt, 1962, page 45 13728.

The concentrations of tin and free acid may be varied generally within the limits conventional in this art. A tin content of 10 to 100 grams per liter, and a free acid concentration of 20 to 200 grams per liter are typical of the sulfate, fluoborate, and aromatic sulfonate solutions, known in themselves, which may be provided with the brighteners of the invention. Sulfuric, fluoboric, and aromatic sulfonic acids may be present simultaneously in the electrolytes in a manner not novel in itself.

55 55 The secondary brighteners which are employed in conjunction with the olefinic primary brighteners in the tin plating solutions of the invention include formaldehyde and certain imidazoline derivatives which may be employed singly or in combination with each other. The imidazoline derivatives which have been found to widen the bright and semi-bright current density range are of

60 60 the formula



70 wherein  $\text{R}_1$  is an alkyl radical with at least 5 carbon atoms,  $\text{R}_2$  is hydrogen or the radical  $-\text{CH}_2-\text{COOH}$ , and  $\text{R}_3$  is hydrogen or a monovalent metal, particularly an alkali

metal. It will be appreciated that the metal may be replaced by hydrogen in the acid electrolyte, and other brighteners of the invention containing carboxyl groups or sulfo radicals may thus be incorporated in the electrolyte in the form of their salts.

Although the imidazoline derivatives described hereinabove are surface active because of the presence of relatively long alkyl chains together with hydrophilic groups, it is preferred to employ them in conjunction with other non-ionic wetting agents. The imidazoline derivatives, however, may replace a portion or all of the formaldehyde which would otherwise be necessary for producing a desired brightening effect.

The amounts of primary and secondary brighteners to be employed vary greatly according to the nature of the substituents present in the primary brightener, and such process variables as the configuration of the object which is made the cathode during the plating process, the desired rate of depositions, and the like. Guidance for the use of the brighteners will be found hereinbelow in the specific examples of embodiments of this invention. Among the secondary brighteners, the imidazole derivatives are effective in concentrations as low as 0.01 gram per liter, and their beneficial effects increase with concentration up to approximately 0.05 to 2.0 grams per liter, the limit varying from compound to compound. At higher concentrations, no further significant improvement is observed, nor are there harmful effects up to the limit of solubility.

Pyrocatechol which is a known antioxidant in acid tin plating solutions, has a beneficial effect when employed in the tin plating solutions of the invention in small amounts.

The temperature of the plating solution is preferably held below 35° C. for best stability, but the maintenance of a specific operating temperature in the tin electrolytes is not critical for the production of bright coatings.

The following examples are further illustrative of the present invention, and it will be understood that the invention is not limited thereto:

#### Example 1

Eight plating solutions were prepared from stannous sulfate, sulfuric acid, formalin (aqueous formaldehyde solution of approximately 37% HCHO content), a polyethyleneglycol wetting agent, and an olefinic brightener as indicated in Table I. The preferred temperature and cathode current density ranges in which smooth, bright tin plates were electrodeposited from the several acid plating solutions are also listed in the table.

The wetting agents employed were ether of polyethoxyethanols which contained approximately 11 C<sub>2</sub>H<sub>4</sub>O radicals in solutions III, IV, and VI, approximately 15 C<sub>2</sub>H<sub>4</sub>O radicals in solutions V, VII, and VIII, 25 C<sub>2</sub>H<sub>4</sub>O radicals in solution II, and 30 C<sub>2</sub>H<sub>4</sub>O radicals in solution I.

- 4
- (III) Furfurylideneacetone or 4-(2-furyl)-3-butene-2-one  
 (IV) o-Methoxycinnamic acid  
 (V) 2-furylacrylic acid  
 (VI) Benzylideneacetone  
 (VII) 2-pentyl-3-phenylpropenal  
 (VIII) Pyridylideneacetone or 4-(pyridyl-2)-3-butene-2-one

The plating solution I was originally somewhat turbid, but became clear after about one day.

#### Example 2

Similar results were obtained with fluoborate bath of the following composition:

|                     | Grams/liter |
|---------------------|-------------|
| Tin (as fluoborate) | 45          |
| Fluoboric acid      | 90          |
| Ether of polyglycol | 2           |
| Formalin            | 1           |
| Cinnamaldehyde      | 0.5         |

The ether of polyglycol employed contained approximately 11 C<sub>2</sub>H<sub>4</sub>O radicals per molecule. The solution gave brightest deposits at temperatures between 20° and 35° C., and at cathode current densities of 1 to 4 amps. per square decimeter. When the cinnamaldehyde was replaced in the plating solution by 0.2 gram/liter benzylideneacetone bright tin deposits were formed under otherwise identical conditions.

#### Example 3

A plating bath was prepared from the following materials:

|                     | Grams/liter |
|---------------------|-------------|
| Stannous sulfate    | 60          |
| Cresolsulfonic acid | 260         |
| Formalin            | 2           |
| Ether of polyglycol | 2           |
| Benzylideneacetone  | 0.4         |

Bright deposits were obtained at 20° to 30° C. over a current density range from 1 to 4 amps. per sq. decimeter. The ether of polyglycol employed as a nonionic wetting agent was the same as in Example 2.

#### Example 4

A tin plating solution that gave a very bright tin electrodeposit at 15° to 30° C. when operated at 1 to 3.5 amps./sq. decimeter has the following composition:

|                     | Grams/liter |
|---------------------|-------------|
| Tin as fluoborate   | 40          |
| Fluoboric acid      | 80          |
| Wetting agent       | 2           |
| Pyridylideneacetone | 0.3         |
| Formalin            | 1           |
| Pyrocatechol        | 1.5         |

TABLE I

| Composition, grams/liter             | Plating Solution No. |       |       |       |         |         |       |       |
|--------------------------------------|----------------------|-------|-------|-------|---------|---------|-------|-------|
|                                      | I                    | II    | III   | IV    | V       | VI      | VII   | VIII  |
| Stannous sulfate                     | 60                   | 60    | 80    | 80    | 60      | 70      | 60    | 80    |
| Sulfuric acid                        | 100                  | 100   | 80    | 120   | 80      | 160     | 120   | 100   |
| Formalin                             | 1                    | 1.5   | 0.8   | 1.6   | 0.8     | 5       | 0.8   | 1     |
| Wetting agent                        | 1                    | 2     | 6     | 5     | 6       | 6       | 6     | 4     |
| Brightener                           | 1                    | 1     | 0.35  | 0.65  | 1.3     | 0.35    | 0.32  | 0.4   |
| Temperature, ° C.                    | 20-30                | 20-30 | 15-30 | 20-30 | 18-30   | 18-30   | 20-30 | 15-30 |
| Current density, amps./sq. decimeter | 1-2.5                | 1-2.5 | 0.8-4 | 1-2.5 | 0.7-3.5 | 0.7-3.5 | 1-2.5 | 1-3.5 |

The following eight brighteners were used in these eight solutions:

- (I) Styrene  
 (II) Cinnamyl alcohol

Less bright, but still very smooth deposits were obtained when the pyrocatechol was omitted from the bath composition. The ether of polyglycol was the same as in Example 2.

## Example 5

A bright tin plating solution was prepared from the following materials:

|                         | Grams/liter |
|-------------------------|-------------|
| Tin as divalent sulfate | 35          |
| Sulfuric acid           | 150         |
| Wetting agent           | 6           |
| Formalin                | 1           |
| Benzylideneacetone      | 0.3         |
| Pyrocatechol            | 0.8         |

At a bath temperature of 20° to 35° C., the bright cathode current density range extended from 1 to 4 amps./sq. decimeter. The wetting agent employed was a ether of polyethylene glycol containing approximately 15 C<sub>2</sub>H<sub>4</sub>O radicals per molecule. Omission of the pyrocatechol from the bath resulted in smooth, but less bright deposits.

## Example 6

Four electroplating solutions were prepared from stannous sulfate, sulfuric acid, a polyethylene glycol wetting agent, an olefinic brightener and a secondary brightener which was an imidazolidine derivative. Pyrocatechol and formalin were used in some of these brighteners. Their compositions, preferred operating temperatures, and the bright plating ranges at these temperatures as listed in Table II.

TABLE II

| Composition, grams/liter                | Plating Solution No. |         |       |       |
|-----------------------------------------|----------------------|---------|-------|-------|
|                                         | IX                   | X       | XI    | XII   |
| Tin (as sulfate)                        | 30                   | 40      | 35    | 35    |
| Sulfuric acid (free)                    | 100                  | 130     | 100   | 150   |
| Wetting agent                           | 6                    | 7       | 6     | 6     |
| Formalin                                | 1.5                  | 0.8     | —     | —     |
| Pyrocatechol                            | —                    | —       | —     | 0.8   |
| Brightener A                            | 0.25                 | 0.4     | 2     | 0.3   |
| Brightener B                            | 0.05                 | 0.6     | 1.0   | 1.0   |
| Temperature, °C.                        | 20-30                | 18-30   | 20-30 | 20-35 |
| Current density amps. per sq. decimeter | 1-4                  | 0.8-3.5 | 1-4   | 1-4   |

The wetting agents in solutions IX to XII had approximately 10-15, 30, 25, 15 C<sub>2</sub>H<sub>4</sub>O radicals per molecule respectively. The olefinic brighteners A were benzylideneacetone (IX and XII), furfurylideneacetone (X), and 2-furylacrylic acid (XI). The imidazolidine derivatives employed as brighteners B may be prepared by the method of U.S. Patents 2,528,378, 2,773,068 and 2,781,354, and were of the formula



in which the substituents were as follows:

|                | IX                              | X                              | XI                              | XII                             |
|----------------|---------------------------------|--------------------------------|---------------------------------|---------------------------------|
| R <sub>1</sub> | C <sub>11</sub> H <sub>23</sub> | C <sub>9</sub> H <sub>10</sub> | C <sub>11</sub> H <sub>23</sub> | C <sub>11</sub> H <sub>23</sub> |
| R <sub>2</sub> | CH <sub>2</sub> -COOH           | H                              | CH <sub>2</sub> -COOH           | CH <sub>2</sub> -COOH           |
| R <sub>3</sub> | H                               | Na                             | H                               | H                               |

A substantial broadening of the bright plating range was achieved by the addition of the imidazolidine derivatives as compared to otherwise identical solutions not containing an imidazolidine derivative. This effect was noticeable not only in the range of fully bright deposits, but also in the semi-bright range. The use of formaldehyde is not absolutely necessary when imidazolidine derivatives are employed as secondary brighteners.

## Example 7

The imidazolidine derivatives of the invention are equally effective as secondary brighteners in tin plating solutions which contain sulfuric, fluoroboric, and aromatic sul-

fonic acids as conductivity increasing and ionization repressing agents. Fully bright tin electrodeposits were obtained from a solution of the following composition under the operating conditions indicated:

|    |                     |              |       |
|----|---------------------|--------------|-------|
| 5  | Tin, as sulfate     | grams/liter  | 30    |
|    | Phenolsulfonic acid | do           | 250   |
|    | Formalin            | do           | 1     |
|    | Benzylideneacetone  | do           | 0.48  |
|    | Wetting agent       | do           | 5     |
| 10 | Brightener B        | —            | 0.8   |
|    | Temperature         | °C           | 20-35 |
|    | Current density     | amps./sq. dm | 1-3.5 |

The wetting agent used was an ether of polyethylene glycol having approximately 15 C<sub>2</sub>H<sub>4</sub>O radicals. The brightener B was an imidazoline derivative of the formula shown in Example 6 in which R<sub>1</sub> was C<sub>7</sub>H<sub>15</sub>, R<sub>2</sub> was CH<sub>2</sub>-COONa, R<sub>3</sub> was sodium. Omission of brightener B from the composition reduced the bright plating range, and particularly the semi-bright plating range.

## Example 8

A stock solution was prepared to the following composition:

|    |                                                                      |             |      |
|----|----------------------------------------------------------------------|-------------|------|
| 25 | Tin (as stannous sulfate)                                            | grams/liter | 30   |
|    | Free sulfuric acid                                                   | —           | 110  |
|    | Ether of polyglycol (abt. 15 C <sub>2</sub> H <sub>4</sub> O groups) | —           | 6    |
|    | Benzylideneacetone                                                   | —           | 0.26 |

30 Three batches of this solution were mixed with the following secondary brighteners respectively:

|    |                            |             |     |
|----|----------------------------|-------------|-----|
| 35 | (a) Formalin               | grams/liter | 1.5 |
|    | (b) Imidazoline derivative | —           | 0.5 |
|    | Formalin                   | —           | 0.8 |
|    | (c) Imidazoline derivative | —           | 1.0 |

The imidazoline derivative employed was the same as in Example 6, IX. The three plating solutions were used at temperatures between 20° and 30° C. and gave at least semi-bright, smooth deposits at cathode current densities from 0.5 to 4 amps. per square decimeter (about 4.5 to 36 amps./sq. ft.). The fully bright range, however, was broadened significantly as the formalin of batch (a) was gradually replaced by the imidazoline derivative.

40 While the invention has been described with particular reference to specific embodiments it is to be understood that it is not limited thereto but is to be construed broadly and restricted solely by the scope of the appended claims.

What we claim is:

50 1. An aqueous acid bright tin electroplating solution including a tin salt, free acid, and as a primary brightener, an effective amount of a compound of the formula X—CH=CH—Y, wherein X is phenyl, furfuryl, or pyridyl, and Y is a member of the group consisting of hydrogen, formyl, carboxyl, alkyl, hydroxyalkyl, formylalkyl, and acyl radicals of carboxylic acids, said compound being dissolved in said aqueous plating solution.

55 2. A solution as set forth in claim 1, further including, as a secondary brightener, an effective amount of at least one member of the group consisting of formaldehyde and imidazoline derivatives of the formula



65 where R<sub>1</sub> is an alkyl radical having at least five carbon atoms, R<sub>2</sub> is a member of the group consisting of hydrogen and —CH<sub>2</sub>-COOH, and R<sub>3</sub> is a member of the group consisting of hydrogen and monovalent metal, said secondary brightener being dissolved in said solution.

70 3. A solution as set forth in claim 2, further including a wetting agent.

4. A solution as set forth in claim 3, wherein said wetting agent is nonionic.

5. A solution as set forth in claim 3, wherein said wetting agent is a water-soluble ether of polyglycol.

6. A solution as set forth in claim 3, wherein X is phenyl.

7. A solution as set forth in claim 3, wherein X is methoxyphenyl.

8. A solution as set forth in claim 3, wherein X is furfuryl.

9. A solution as set forth in claim 3, wherein X is pyridyl.

10. A solution as set forth in claim 3, wherein Y is the acyl radical of a carboxylic acid.

11. A solution as set forth in claim 5, wherein X is sulphonylphenyl.

12. A solution as set forth in claim 5, further including pyrocatechol as an antioxidant.

13. A method of electrodepositing bright tin on an article which comprises making said article the cathode in an aqueous solution including a soluble tin salt, free acid, a nonionic wetting agent, and effective amounts of primary and secondary brighteners, said primary brightener being a compound of the formula  $X-CH=CH-Y$ , wherein X is phenyl, furfuryl, or pyridyl, and Y is a member of the group consisting of hydrogen, formyl, carboxyl, alkyl, hydroxalkyl, formylalkyl, and acyl radicals of carboxylic acids, said compound being dissolved in said aqueous plating solution, and said secondary brightener including at least one member of the group

consisting of formaldehyde and imidazoline derivatives of the formula



wherein  $\text{R}_1$  is an alkyl radical having at least five carbon atoms,  $\text{R}_2$  is a member of the group consisting of hydrogen and  $-\text{CH}_2\text{---COOH}$ , and  $\text{R}_3$  is a member of the group consisting of hydrogen and monovalent metal, said secondary brightener being dissolved in said solution.

14. A method as set forth in claim 13, wherein said wetting agent is a water soluble ether of polyglycol.

15. A method as set forth in claim 13, wherein said free acid is selected from the group consisting of sulfuric acid, fluoboric acid, and phenolsulfonic acids.

16. A method as set forth in claim 13, wherein said solution is at a temperature not substantially higher than  $35^\circ \text{C}$ .

#### References Cited

##### UNITED STATES PATENTS

2,598,486 5/1952 Andrews ----- 204-54

25 3,082,157 3/1963 Francisco et al. ----- 204-54

ROBERT K. MIHALEK, Primary Examiner.

JOHN H. MACK, Examiner.

30 G. KAPLAN, Assistant Examiner.